

March 3, 1942.

L. J. DYKSTRA ET AL  
HIGH TENSION ELECTRIC INSULATOR AND METHOD OF  
ATTACHING A METAL FITTING THERETO  
Filed Sept. 17, 1940

2,274,954



INVENTORS.  
Laurence J. Dykstra  
Edwin M. Meyer  
Harold L. Stonebraker  
BY their Attorney

## UNITED STATES PATENT OFFICE

2,274,954

HIGH TENSION ELECTRIC INSULATOR AND  
METHOD OF ATTACHING A METAL FIT-  
TING THERETOLaurence J. Dykstra and Edwin M. Meyer, Roch-  
ester, N. Y., assignors to Victor Insulators, Inc.,  
Victor, N. Y., a corporation of New York

Application September 17, 1940, Serial No. 357,162

16 Claims. (Cl. 174—158)

This invention relates to a high tension electric insulator and method of attaching a metal fitting thereto, and has for its object to afford a practical and economical procedure for effecting a bond between a silica-containing insulator body, such as porcelain, and a metal fitting such as a surrounding steel ring adapted to be secured to a structure where the insulator is to be used.

More particularly, the invention is intended to afford a stronger and more durable bond between metal and silica-containing surfaces than has heretofore been commercially practicable, and a joint between such parts which constitutes a tight and effective hermetic seal against any cold or hot liquid or gaseous medium.

A more specific purpose of the invention is to provide means for firmly uniting a steel or similar metal ring to a cylindrical hollow porcelain insulator body such as employed for condenser and pothead bushings where a conductor extends through the porcelain unit, and a liquid-tight joint between the metal ring and porcelain unit is required.

To these and other ends, the invention consists in the construction and method that will appear clearly from the following description when read in conjunction with the accompanying drawing, the novel features being pointed out in the claims following the specification.

The drawing is a sectional view of an insulator, constructed in accordance with a preferred embodiment of the invention.

Referring more particularly to the drawing, 1 designates a hollow, generally cylindrical insulator body of suitable silica-containing material, preferably porcelain, and having the usual silicate glazed outer surface, 2 is a steel, cast iron, or other suitable metallic ring or collar having an exteriorly threaded portion 3 adapted to engage a threaded opening in a tank or support, and 4 designates an interiorly threaded portion on the metal ring for obtaining a firmer mechanical bond. 5 designates a body of antimony between the porcelain surface and the interior of the metal ring, the antimony acting to cause the latter to adhere tightly to the porcelain by forming an alloy with the silica in the insulator body as well as the metal ring, and effecting a liquid-tight joint therebetween.

In the structure shown, 6 designate a series of annular ribs or projecting portions, the uppermost one terminating in a shoulder upon which an asbestos gasket 7 is placed during the attaching of the metal ring, in order to space

the latter from the porcelain shoulder and prevent direct contact, which might result in fracturing the porcelain upon expansion or contraction of the parts.

5 To attach a ring to a porcelain body in this fashion, the insulator or porcelain body, either with or without the usual silicate glaze covering it, is first fired, or subjected to the usual heat treatments necessary to finish a porcelain insulator. Such a fired insulator, after having cooled to normal room temperature, is placed in a furnace in the position shown, with the metal ring 2 resting upon the asbestos spacing element 7, and heated preferably over a period of about four 10 hours to 1250° F. to 1300° F., such gradual increase in temperature protecting the porcelain against damage from too sudden application of excessive heat, or the porcelain may be heated to a lesser degree, but sufficiently to eliminate 15 thermal shock when molten antimony is brought into contact with it.

When the porcelain reaches a proper temperature, molten antimony, previously melted in any suitable manner, is poured between the ring 2 and the porcelain, as indicated at 5, and the parts, with the antimony filling the space between the metal ring and the porcelain, are permitted to remain in the furnace for approximately 20 from forty-five minutes to one hour and a quarter, the heating process being carried on in a reducing atmosphere, as by charging the furnace with charcoal, in order to prevent oxidation of the antimony. The antimony may be introduced between the ring and porcelain in powdered or lump form, and the entire assembly, 25 including the porcelain, ring, and antimony, raised to the required temperature at the same time.

The antimony thus remains in a metallic state, 30 being protected against oxidation, and there is probably formed an alloy of silica and antimony, due to softening of the silica in the porcelain or the silicate glaze thereon. Whatever the action between the antimony and silica, there is 35 formed an intimate and strong mechanical bond between the metal ring and the porcelain that effectually prevents separation of these parts, and serves as a perfect seal against the passage through the joint of either hot or cold liquid or 40 gas. This is particularly essential where such a bushing is employed with a condenser, cable terminal, pothead, or capacitor that is filled with hot oil which is under pressure, and it is necessary to prevent leakage of such hot oil between 45 the ring 3 and the insulator body. It will be 50

understood that the threaded portion 3 of the ring is secured in an opening in the condenser tank or housing, and the hollow insulator bushing through which the conductor passes is sealed at its outer end, the inner end extending into the condenser tank and receiving the conductors.

With this procedure and such use of antimony, it is possible to obtain a stronger mechanical bond between a silica-containing surface and a metal fitting than with any known cements or adhesives that depend upon cohesion between rough surfaces for their union, and it has been determined by actual tests that with a joint such as described, the porcelain will fracture before separating from the antimony bond. While it is not known with certainty what action takes place, it is believed that the antimony forms an alloy with both the metal ring and the porcelain body, flowing into and intermingling intimately with said surfaces so that there is a mechanical overlapping and molecular bond between the antimony layer and both the porcelain and metal surfaces, resulting in an integral union as distinguished from a mere cementing together of two opposed surfaces.

While the invention has been described with reference to a particular type of insulator, it is not confined to this form only, but may be otherwise utilized wherever it is desirable to unite a metal fixture to a silica-containing insulator body, and both the structure and method may be modified without departing from the essential features of the invention and the scope of the following claims.

We claim:

1. In a high tension electric insulator, the combination with a silica-containing body, of a metal fitting, and an integral molecular bond of antimony uniting the metal fitting and the silica-containing body.
2. In a high tension electric insulator, the combination with a porcelain body, of a metal fitting, and an integral molecular bond of antimony uniting the metal fitting and the porcelain body.
3. In a high tension electric insulator, the combination with a porcelain body having a silicate glaze, of a metal fitting, and an integral molecular bond of antimony uniting the metal fitting and glazed porcelain body.
4. In a high tension electric insulator, the combination with a silica-containing body, of a metal ring surrounding the silica-containing body, and an integral molecular bond of antimony between the ring and silica-containing body.
5. In a high tension electric insulator, the combination with a porcelain body, of a metal ring surrounding the porcelain body, and an integral molecular bond of antimony between the ring and porcelain body.
6. In a high tension electric insulator, the combination with a porcelain body having a silicate glaze, of a metal ring surrounding the glazed porcelain body, and an integral molecular bond of antimony between the ring and glazed porcelain body.
7. In a high tension electric insulator, the combination with a porcelain body, of a metal fitting, and an alloy of silica and antimony constituting an integral molecular bond between the metal fitting and porcelain body.
8. The method of attaching a metal fitting to a silica-containing insulator body which consists in first firing the insulator body, and then apply-

ing molten antimony between the fitting and the insulator body while maintaining the insulator body at the temperature of the molten antimony, approximately from 1250° F. to 1300° F.

9. The method of attaching a metal fitting to a porcelain insulator body which consists in first firing the insulator body and then applying molten antimony between the fitting and the insulator body while maintaining the insulator body at the temperature of the molten antimony, approximately from 1250° F. to 1300° F.

10. The method of attaching a metal fitting to a porcelain insulator body having a silicate glaze which consists in first firing the glazed porcelain body and then applying molten antimony between the fitting and the insulator body while maintaining the insulator body at the temperature of the molten antimony, approximately from 1250° F. to 1300° F.

11. The method of attaching a metal ring to a silica-containing insulator body which consists in first firing the silica-containing insulator body, positioning the ring around the insulator body in spaced relation thereto, and applying molten antimony between the ring and the insulator body while maintaining the insulator body at the temperature of the molten antimony, approximately from 1250° F. to 1300° F.

12. The method of attaching a metal ring to a porcelain insulator body which consists in first firing the porcelain insulator body, positioning the ring around the insulator body in spaced relation thereto, and applying molten antimony between the ring and the insulator body while maintaining the insulator body at the temperature of the molten antimony, approximately from 1250° F. to 1300° F.

13. The method of attaching a metal ring to a porcelain insulator body having a silicate glaze which consists in first firing the glazed insulator body, positioning the ring around the insulator body in spaced relation thereto, and applying molten antimony between the ring and the insulator body while maintaining the insulator body at the temperature of the molten antimony, approximately from 1250° F. to 1300° F.

14. The method of attaching a metal fitting to a silica-containing insulator body which consists in first firing the insulator body, and arranging molten antimony between the metal fitting and the insulator body while heating the insulator to the melting point of the antimony, approximately from 1250° F. to 1300° F.

15. The method of attaching a metal ring to a silica-containing insulator body which consists in first firing the insulator body, positioning the ring around the insulator body in spaced relation thereto, and arranging molten antimony between the metal ring and the insulator body while heating the porcelain to the melting point of the antimony, approximately from 1250° F. to 1300° F.

16. The method of attaching a metal ring to a porcelain insulator body having a silicate glaze which consists in first firing the glazed insulator body, positioning the ring around the insulator body in spaced relation thereto, and arranging molten antimony between the metal ring and the insulator body while heating the porcelain to the melting point of the antimony, approximately from 1250° F. to 1300° F.

LAURENCE J. DYKSTRA.  
EDWIN M. MEYER.